# EUROPEAN PATENT SPECIFICATION

(11) **EP 0 098 025 B1**
(45) Date of publication and mention of the grant of the patent: **24.05.1989**
(21) Application number: 83200964.1
(22) Date of filing: 28.06.1983
(51) Int. Cl.: D01F 9/22

(54) **Process for producing polyacrylonitrile-based carbon fiber**
Verfahren zur Herstellung von aus Polyacrylnitril hergestellten Kohlenstoffasern
Procédé de production de fibres de carbone à base de polyacrylonitrile

(30) Priority: 29.06.1982 US 393392
(43) Date of publication of application: 11.01.1984
(73) Proprietor: AMOCO CORPORATION, Chicago Illinois 60680 (US)
(72) Inventor: Schulz, David Arthur, Fairview Park Ohio 44126 (US)
(74) Representative: van der Beek, George Frans, Ir.

(56) References cited:
- DE-A- 2 130 600
- FR-A- 1 558 690
- FR-A- 1 581 203
- FR-A- 2 009 894

## Description

The commercial value of polyacrylonitrile(PAN)-based carbon fibers is well known in the prior art.

Generally, a PAN-based carbon fiber is produced by spinning polyacrylonitrile into a fiber, infusibilizing the fiber by raising it to an elevated temperature in air, and thereafter carbonising the infusibilized fiber at an elevated temperature in an inert atmosphere under tension in a threadline to produce a carbon fiber.

Commercially, thousands of continuous filaments or fibers are spun simultaneously and collected together to form a green yarn and the yarn is processed subsequently to produce an infusibilized yarn and then a carbon yarn.

The carbonizing opeation for the infusibilized yarn is carried out as a threadline operation in order to subject the yarn to tension during the carbonising step. The carbonizing step can be carried out as a sequence of operations using separate heating units. For example, one heating unit can be used at a temperature of about 1300°C to carbonize the infusibilized yarn initially and another heating unit can be used to carbonize the yarn to a higher temperature and thereby improve the mechanical properties of the carbon yarn. (cf. e.g. FR-A-1,558,690 and FR-A-2,009,894).

One of the drawbacks of the prior art processes for commercially producing PAN-based carbon yarns is that the tensile strength of the fibers degrades as the carbonising processing results in a higher Young's modu!us. Table I shows typical properties of commercially available PAN-based carbon fibers.

In contrast, the instant invention produces a PAN-based carbon yarn having as average fiber properties a Young's modulus of greater than about 344.10⁶ kPa and a tensile strength at least one third greater than the commercially available PAN-based carbon fiber having a similar average value of Young's modulus.

In addition, the process according to the invention is simple to implement and can be carried out economically with improved productivity, yielding high quality PAN-based carbon fibers.

The process of the invention for preparing PAN-based carbon fiber is characterized by the steps of 1
a. heating an infusibilized PAN fiber on a bobbin (which is of course thermally and mechanically stable at the heating temperature and which is chemically compatible with the infusibilized fiber) at a rate of 50° to 500°C per hour to a temperature in the range of from about 1300 to 1700°C;
b. holding the fiber at a temperature within the range until the elemental nitrogen content of the fiber is at most 1 wt. percent and
c. further heating the fiber to a temperature of 1900°C or above.

Preferably the above step c is carried out in a threadline operation. However, it is also possible to obtain carbon fibers having both a high Young's modulus and a satisfactory tensile strength is said step c is carried out completely integrated with the above steps a and b as explained in Example 3 hereinbelow. That means that the infusibilized PAN fiber is heatged on a bobbin first according to the requirement of step a, thereafter according to the requirement of step b and finally according to the requirement of step c. ' Step c is preferably carried out in an inert atmosphere.

For commercial operations, the process would be carried out using yarn, a plurality of fibers.

The bobbin for carrying out the process comprises a cylindrical body made of material such as stainless steel, or refractory oxides, or boron nitride, or graphite and preferably has a layer of compressible resilient carbon material such as carbon felt positioned on the outside surface of the cylindrical body to receive the infusibilized fiber and thereby minimize the stress between the cylindrical body and the infusibilized fiber during the treatment. The bobbin can be with or without end flanges. For relatively high winding angles, and flanges are not needed.

Typically, the cylindrical body of the bobbin can have an inside diameter of 7.62 cm and an outside diameter of about 8.89 cm with an overall length of about 27.94 cm.

Preferably, carbon felt has a thickness of from about 0.63 cm to about 1.27 cm thick.

The winding of the infusibilized yarn onto a bobbin can be carried out using a range of winding angles. Preferably a wind angle of at least two degrees should be used and as high as about twenty-three degrees is advantageous. During the heat treatment on the bobbin, the fibers tend to shrink considerably and the use of a high wind angle permits shrinkage without adverse effects on the fibers. Moreover, the use of a high wind angle leads to uniform fiber properties throughout the length of the fiber from the core to the outer winding layer.

The heat treatment of the fibers on the bobbins conveniently allows the bulk heat treatment of a large amount of fibers, at a relatively slow rate of increase in temperature to an elevated final temperature. The surprising advantage of this heat treatment is that both the rate of reduction in nitrogen content of the fibers and the final nitrogen content are much lower as to compared to a heat treatment to the same final temperature using a conventional threadline arrangement. As a result the subsequent threadline heat treatment can be carried out at a high rate of movement of the yarn through the heating unit even if a considerably elevated temperature is used. This threadline treatment straightens out the fibers and establishes the final fiber mechanical properties.

Generally, the threadline temperature should be at least about 600°C higher than the temperature used for the first heat treatment of the yarn on the bobbin.

Table II shows a typical schedule of temperatures for the first and second heat treatments according to the invention in order to obtain PAN-based carbon fibers having predetermined values for the Young's modulus. The estimated nitrogen content after the first heat treatment is an important criteria for determining the heat of the threadline for any given temperature for the second heat treatment. A high nitrogen content will result in severe fiber damage due to the sudden evolution of the nitrogen from the fiber during a sudden temperature increase for a second heat treatment.

Generally, the first heat treatment according to the invention is carried out at a rate of from about 50°C to about 500°C per hour to a maximum temperature of from about 1300°C to about 1700°C.

Preferably, the first heat treatment is carried out by increasing the temperature at the rate of about 50°C for an hour from room temperature to about 800°C and thereafter increasing the temperature at a rate of 250°C per hour until the predetermined maximum temperature is reached and the maximum temperature is maintained for an additional two hours. The maximum temperature is maintained in order to give all of the fibers on the bobbin the opportunity to reach a temperature equilibrium.

A typical prior art threadline heat treatment at a temperature of 1300°C results in a PAN-based carbon fiber having a nitrogen content of about 4% or more by weight whereas the same heat treatment carried out using the first heat treatment according to the invention results in a PAN-based carbon fiber having a nitrogen content of about 1 % by weight. The lower nitrogen content is important for carrying out a second heat treatment using a threadline at a relatively high speed.

For a fuller understanding of the nature of objects of the invention, reference should be had to the following detailed description, taken in connection with the accompanying drawings, in which:
Fig. 1 is a graph showing the effect of a first heat treatment according to the invention on the chemical composition of PAN-based fibes;
Fig. 2 is a graph showing the effect of threadline temperature and line speed on the density of recarbonized conventional PAN-based carbon fibers;
Fig. 3 is a graph showing the effect of line speed on threadline temperature on the density of recarbonized conventional PAN-based carbon fibers;
Fig. 4 is a graph comparing the effect of threadline temperature on the density of recarbonised conventional PAN-based carbon fibers and recarbonized PAN-based carbon fibers produced according to the instant invention;
Fig. 5 is a graph showing the effect of threadline temperature and line speed on the tensile strength of recarbonized PAN-based carbon fibers;
Fig. 6 is a graph showing a comparison of the effect of threadline temperature on the tensile strength of both recarbonised conventional PAN-based carbon fibers and recarbonized PAN-based carbon fibers produced according to the instant invention;
Fig. 7 is a graph comparing the effects of threadline temperature and line speed on the Young's modulus of both recarbonised conventional PAN-based carbon fibers and recarbonized PAN-based carbon fibers produced according to the instant invention;
Fig. 8 is a graph showing a comparison of the tensile strength versus Young's modulus for both recarbonized conventional PAN-based carbon fibers and recarbonized PAN-based carbon fibers produced according to the invention;
Fig. 9 is a graph showing a comparison between the tensile strength versis Young's modulus for both recarbonised PAN-based carbon fibers and recarbonized PAN-based carbon fibers produced according to the invention.

In carrying out the invention, certain embodiments have been selected for description in the specification and reference is had to the Fig. 1 to 9.

It is economical in the commercial production of PAN-based carbon yarns to carry out the carbonising operation in two separate steps. The first step is a carbonising in a threadline to a temperature of about 1300°C while the second step is a threadline operation at a higher temperature to improve the mechanical properties of the resulting carbon yarn.

Subjecting an infusibilized fiber to a heat treatment results in the release of nitrogen, oxygen, and hydrogen from the fiber. Fig. 1 shows the weight percent of the aforementioned gases and carbon as a result of a first heat treatment in accordance with the invention. The reduction in nitrogen content is particularly important because the loss of nitrogen during a subsequent threadline heat treatment at a higher temperature can result in serious degradation of the fibers.

The tests for Fig. 1 were carried out using a graphite bobbin wrapped with a single layer of graphite felt and the temperature was increased from room temperature to the final temperature at the rate of about 100°C per hour with the final temperature as shown being held for two hours.

In addition to the substantial reduction in nitrogen content, it is significant that the evolution of nitrogen was at a relatively slow rate, particularly in comparison to a threadline operation ar 1300°C. It is important that the evolution of nitrogen be at a slow rate so that the escaping gases will not produce flaws and degradation in the quality of the fibers.

Fig. 2 shows the results of a second heat treatment using a threadline operation for fibers which have been subjected to a first heat treatment using a conventional threadline operation at a temperature of about 1300°C. The loss in the density of the carbon fibers for high speeds through the furnace is due to the almost explosive evolution of nitrogen.
Fig. 3 presents the data of Fig. 2 in a different arrangement. From Figs. 2 and 3 it is evident that a threadline heat treatment of a PAN-based fiber which has been subjected to a previous threadline heat treatment has limitation as to the threadline speed and maximum treatment temperature.
Fig. 4 is a comparison in the fiber density after a threadline heat treatment of a fiber which has been subjected to a prior art threadline heat treatment and a fiber which has been subjected to the first heat treatment in accordance with the invention. In both cases, the first heat treatment had a maximum temperature of 1300°C. The line speed the second heat treatment in both cases was maintained at 1829 cm per minute. The evident degradation in fiber density is a result of the rapid evolution of nitrogen. The fiber given a first heat treatment in accordance with the invention has a very low nitrogen content.
Fig. 5 shows the effect of second conventional threadline temperature and line speed on the tensile strength of recarbonised PAN-based carbon fibers which have been subjected to a first conventional threadline treatment. The tensile strength declines rapidly in each case even for relatively slow line speeds as the maximum heat treatment temperature increases.
Fig. 6 shows the tensile strength of fibers after being subjected to a second heat treatment using a conventional threadline. The fiber which has been given a first heat treatment in accordance with the invention is significantly better than the fiber which has been subjected for a first heat treatment in accordance with the prior art. The line speed in all cases was 1219 cm per minute.
Fig. 7 shows the Young's modulus versus maximum temperature for a second heat treatment using a conventional threadline for fibers having a first heat treatment according to the invention and for fibers having a heat treatment according to the prior art. The first heat treatment in all cases had a maximum temperature of 1300°C. The carbon fibers according to the instant invention consistently showed higher value for the Young's modulus even when the line speed for the second heat treatment was ten times greater than the line speed used for the fibers according to the prior.art.
Fig. 8 shows the relationship for tensile strength and Young's modulus for fibers according to the instant invention and prior art. In each case, the first heat treatment was carried out using a maximum temperature of 1300°C while the second heat treatments were both convention threadline operations. For both operations, the same threadline speed was used and different temperatures were used to obtain various fiber properties. The data show that for each Young's modulus the tensile strength of the fibers produced by the instant invention is substantially higher than the tensile strength of the fibers produced according to the prior art.
Fig. 9 shows a comparison between the tensile strength and the Young's modulus for fibers prepared according to the instant invention and the prior art. In each case, the maximum temperature used for the first heat treatment was 1300°C and the maximum temperature used in the second heat treatment was 1900°C. The variations in mechanical properties were produced by changes in threadline speed. The carbon fibers according to the invention were overwhelmingly superior to the fibers produced according to the prior art.

Illustrative, non-limiting examples of the practice of the invention are set out below. The parts and percentages as cited herein and all through the specification, unless specifically stated otherwise, refer to parts by weight and percentages by weight.

### Example 1 (comparative example)

A PAN-based infusibilized yarn was used. The fibers in the yarn had a composition of 64.0% carbon, 3.9% hydrogen, 6.2% oxygen, and 25.1 % nitrogen. The yarn was wound on a bobbin used in commercial production. The yarn was unwound from the bobbin and rotated at 500 revolutions per minute while being unwound at the rate of 1920 cm per minute so that a twist of 0.7 turns per 2.54 cm was established. The twisted yarn was rewound with a tension of 250 grams onto a graphite bobbin having dimensions of 0.89 cm in diameter and 27.94 cm long. The grpahite bobbin had a layer of 0.63 cm of graphite felt on the cylindrical portion to receive the yarn. A wind angle of 23 degrees was used and the package pressure was 1.36 kg with a transverse length of 25.4 cm. The rewound yarn amounted to 7163 m of yarn and was in the form of a square-sided package.

The package was placed horizontally in a graphite tube induction furnace which was purged with nitrogen and fired at the rate of 50°C per hour to 800°C and thereafter temperature was raised at 250°C per hour to 1300°C. The final temperature was maintained for two hours and the package was allowed to cool back to room temperature. As a result of the heat treatment, the package had shrunk longitudinally about 3.81 cm to 5.08 cm from its original 25.4 cm length. The elemental nitrogen content was 0.9%.

The package was then mounted horizontally on a tension-loaded payoff creel, and the yarn was unwound under a tension of approximately 50 grams, passed through a grooved-reel, tension-controlled drive system maintained at a tension of about 1.825 grams and thereafter through grpahite tube electric resistance furnace having a hot zone maintained at a temperature of about 1830°C and 152 cm long. The yarn exiting the furnace was then subjected to a finish treatment in accordance with the prior art and wound onto bobbins made of cardboard in 305 m lengths. Twenty-two samples of the yarn were taken at about 305 m intervals.

The average tensile strength of the resulting fiber was 3447.10³ kPa with a coefficient of variation of 1.3%. The average Young's modulus for the resulting fiber was about 284.10⁶ kPa with a coefficient of variation of 2.9%. The average density of the fibers was 1.766 Mg per cubic meter with a coefficient of variation of 0.6%. The average yield was 2397 m per kg with a coefficient of variation of 2.1%.

The carbon yarn obtained had an excellent appearance and was equivalent in quality to a carbon yarn produced by carbonizing with two separate threadlines in accordance with the prior art.

### Example 2

Infusibilized yarn as in Example 1 was used in this example. For this example, however, 1432 m on infusibilized yarn was used. As in Example 1, the yarn was wound onto the graphite bobbin having a graphite felt layer.

The same temperature schedule was used for the first heat treatment. The second heat treatment was different in this example for Example 1 in that the furnace temperature was held at 2460°C, the take off tension was 100 grams, the line tension was 1950 grams, the line speed was 2134 cm per minute, and only water was applied to the carbon yarn instead of a finish.

Five samples taken at about equal separations were tested. The fibers had an average tensile strength of 3289.10³ kPa, an average Young's modulus of 391.10⁶ kPa, a density of 1.813 Mg per cubic meter, and a yield of 2549 m per kg. The yarn was excellent in appearance.

### Example 3

1432 m of carbon yarn produced from the steps of Example 1 were wound on a graphite bobbin having a diameter of 11.43 cm and a length of 17.78 cm. No carbon felt was used and the wind angle was about 0.4°. This package was then loaded horizontally in a graphite tube induction furnace, purged with argon, and fired at the rate of 100°C per hour to a temperature of 2950°C. The final temperature was maintained for two hours and the package was allowed to cool back to room temperature.

The average properties of the fibers so obtained was a tensile strength of 2482.10³ kPa, Young's modulus of 668.10⁶ kPa, density of 2.080 Mg per cubic meter, and a yield of 2832 m per kg. The reduction in strength over the values obtained from Example 1 indicates that new flaws were introduced during the subsequent thermal processing and handling.

In any event, the carbon fibers of this example constitute a significant improvement over commercially available PAN-based carbon fibers.

## Claims

A process for preparing PAN-based carbon fiber characterized by the steps of
a. heating an infusibilized PAN fiber on a bobbin at a rate of 50° to 500°C per hour to a temperature in the range of from about 1300 to 1700°C;
b. holding the fiber at a temperature within that range until the elemental nitrogen content of the fiber is at most 1 wt. percent and
c. further heating the fiber to a temperature of 1900°C or above.

## Patentansprüche

Verfahren zur Herstellung einer Kohlenstoffaser auf PAN-Basis, gekennzeichnet durch die Schritte:
a. Erhitzen einer unschmelzbar gemachten PAN-Faser aus einer Spule mit einem Anstieg von 50 bis 500°C pro Stunde bis auf eine Temperatur im Bereich von etwa 1300 bis 1700°C;
b. Halten der Faser auf einer Temperatur innerhalb dieses Bereichs bis der Gehalt der Faser an elementaren Stickstoff höchstens 1 Gew.% beträgt und
c. weiteres Erhitzen der Faser auf eine Temperatur von 1900°C oder darüber.

## Revendications

Procédé de préparation d'une fibre de carbone à base de PAN, caractérisé par les étapes consistant:
a. à chauffer une fibre de PAN rendue infusible sur une bobine à une vitesse de 50° à 500°C par heure jusqu'à une température comprise dans l'intervalle d'environ 1300° à 1700°C;
b. à maintenir la fibre à une température comprise dans cet intervalle jusqu'à ce que la teneur en azote élémentaire de la fibre soit au maximum de 1 % en poids et
c. à poursuivre le chauffage de la fibre jusqu'à une température de 1900°C ou au-dessus.
